

## UNITED STATES PATENT OFFICE

2,599,424

## MANUFACTURE OF AN ACRYLIC ACID ESTER

Otto Albrecht, Muenchenstein, and Arthur Maeder, Basel, Switzerland, assignors to Ciba Limited, Basel, Switzerland, a Swiss firm

No Drawing. Original application February 12, 1948, Serial No. 7,998. Divided and this application June 19, 1950, Serial No. 169,071. In Switzerland February 21, 1947

10 Claims. (Cl. 260—405)

1

This application is a division of abandoned application Ser. No. 7,998, filed February 12, 1948.

According to this invention esters of olefine carboxylic acids are made by treating a compound of the acetylene series with nickel carbonyl or cobalt carbonyl with the addition of an acid and of a hydroxy compound which contains at least one alcoholic hydroxy group and at least one carbon chain with at least 12 carbon atoms. In this manner there are obtained from compounds containing the grouping  $-\text{C}\equiv\text{C}-$  esters containing the grouping



in which  $-\text{OR}$  represents the residue of the hydroxy compound used having the formula  $\text{HOR}$ , or mixtures of such an ester with the free olefine carboxylic acid. With acetylene there are obtained by this process esters of acrylic acid or mixtures of acrylic acid esters and free acrylic acid.

As a compound of the acetylene series acetylene itself is the preferred starting material. However, there may also be used as starting materials substituted acetylenes, such as methyl-acetylene, ethyl-acetylene, phenyl-acetylene, vinyl-acetylene, divinyl-acetylene, isopropenyl-acetylene, 1-ethinyl-cyclohexene-(1)-; and also alkinols or alkyne-diols such as butine-(1)-ol-(4), pentene-(3)-ine-(1)-ol-(5), and also ethers or esters thereof or products obtainable therefrom by dehydration; furthermore ketones of the acetylene series, such as hexene-(3)-ine-(5)-one-(2); also propiolic acid esters or other acetylene carboxylic acid esters, such as stearolic acid esters, dehydro-undecylenic acid esters, undecolic acid esters, behenolic acid esters. There are also to be mentioned among acetylene compounds which may be used as starting materials alkinols derived from steroid ketones, such as testosterone, or from tetralones, by the addition of acetylene.

Among the hydroxy compounds which contain at least one alcoholic hydroxy group and at least one carbon chain with at least 12 carbon atoms to be used as starting materials in the invention there may be mentioned the following alcohols: Laurin alcohol, cetyl alcohol, octadecyl alcohol, montan alcohol; further the following hydroxyl compounds: Hydroxy-carboxylic acids such as ricinoleic acid or the hydroxy-stearic acid obtainable by the hydrogenation of ricinoleic acid; esters and amides of hydroxy-carboxylic acids, such as octadecyl glycolate, methyl ricinoleate,

2

octadecyl ricinoleate, castor oil, 11-hydroxy-stearic acid cetyl ester, 11-hydroxy-stearic acid amide; polyhydric alcohols partially esterified with carboxylic acids, especially higher fatty acids, such as lauric acid  $\beta$ -hydroxy-ethyl ester, stearic acid  $\beta$ -hydroxyethyl ester, behenic acid  $\beta$ -hydroxyethyl ester, montanic acid  $\beta$ -hydroxyethyl ester, mono- or diglycerides of higher fatty acids, for example, of stearic acid, oleic acid, linoleic acid or linolenic acid, such as linseed oil fatty acid monoglyceride or linseed oil fatty acid diglyceride; hydroxyalkyl amides of higher fatty acids, such as stearic acid  $\beta$ -hydroxyethylamide; further hydroxy-alkyl-thioethers such as  $\beta$ -hydroxy-ethyl-dodecyl-thioether.

There may be used as acids in the present invention, for example, hydrohalic acids, especially hydrochloric acid, but also phosphoric acid or acetic acid. They are advantageously used in aqueous solution.

The reaction of the invention may be carried out by mixing the reactants together at room temperature or at a raised temperature, if desired, in a pressure vessel. When acetylene and nickel carbonyl are used as starting materials the reaction may be carried out at room temperature or a moderately raised temperature, for example, at 30–30° C. under atmospheric pressure or under superatmospheric pressure. For example, acetylene may be introduced into a mixture of the hydroxy compound and the acid and the nickel carbonyl introduced dropwise at the same time. It is still more advantageous to mix the hydroxy compound, acid and nickel carbonyl together, if desired, with the addition of a solvent, preferably an inert one, and to agitate the mixture with acetylene in a suitable agitating apparatus under slightly superatmospheric pressure. Substituted acetylenes of lower reactivity, for example, alkinols, are advantageously reacted with the metal carbonyl, especially nickel carbonyl, at a raised temperature, for example, at 50–120° C., the use of the easily volatile nickel carbonyl making it necessary to work in a pressure vessel.

For the purpose of working under atmospheric pressure there are used for 1 mol of the acetylene compound at least  $\frac{1}{4}$  mol of nickel carbonyl or cobalt carbonyl, at least  $\frac{1}{2}$  mol of a monobasic acid and at least 1 mol of the hydroxy compound. When the reaction is conducted in a pressure vessel at a raised temperature, for example, at 120–150° C., the quantity of the metal carbonyl may be reduced, but carbon monoxide must be present in excess. It is also possible to form the metal carbonyl during the reaction,

when the latter is conducted at a raised temperature and under pressure, by working in the presence of metallic nickel or cobalt or a salt thereof, especially a halide, with the addition of an excess of carbon monoxide. In this case only small quantities of nickel or cobalt or a salt thereof are necessary, as these additions act as catalysts.

The process may be conducted discontinuously or continuously.

As already stated the products of the invention consist predominantly of esters of carboxylic acids which contain a double bond in the  $\alpha:\beta$ -position, if desired, in admixture with the carboxylic acids from which the esters are derived. When necessary, the free olefine carboxylic acids present in the reaction mixture may be subsequently esterified. This may be brought about in the usual manner, for example, by distilling off the water present in the reaction mixture, and heating the mixture containing the olefine carboxylic acid and the alcohol until the esterification ceases. The water may be removed during the esterification azeotropically or, in the case of high boiling alcohols, by evacuation.

Owing to the reactive double bond the products of the invention are suitable, for example, as intermediate products, for instance, for the manufacture of polymerisates. The acrylic acid esters obtainable, for example, from acetylene, polymerise with the application of heat, especially in the presence of a polymerisation accelerator, such as benzoyl peroxide, whereby polymerisates are obtained whose properties depend on the choice of the starting materials.

Such polymeric acrylic acid esters can be used for producing coatings on textiles or paper, and also as artificial substances or adhesives or as constituents of lacquers, artificial masses or the like. Acrylic acid esters obtained by the invention and containing an aliphatic residue of at least 16 carbon atoms can be used, either in monomeric or polymeric form, for improving textiles, especially for dressing them and imparting hydrophobic properties thereto. To this end the textiles may, for example, be impregnated with solutions of the polymeric ester in organic solvents or with aqueous dispersions thereof, and dried at a raised temperature. Alternatively, suitable monomeric acrylic acid esters, especially those which polymerize easily, may be applied to the textile material, and polymerized on the fiber at a raised temperature in the presence of a substance which accelerates the polymerisation.

The following examples illustrate the invention, the parts being by weight unless otherwise stated, and the relationship of parts by weight to parts by volume being the same as that of the kilogram to the liter:

#### Example 1

74 parts of hardened castor oil are dissolved with heat in a mixture of 135 parts of benzene and 115 parts of benzine. The warm solution, after the addition of 18 parts of concentrated hydrochloric acid (density=1.199) and 10 parts of nickel carbonyl, is agitated with acetylene until the gas is no longer absorbed. At the outset the color changes towards dark brown, and as the reaction proceeds the color becomes pale again and solid  $\text{NiCl}_2$  separates, while there is a considerable spontaneous liberation of heat.

After cooling, the whole is filtered to remove the precipitated nickel chloride, and the solvent

is removed by distillation under reduced pressure.

There are obtained 80 parts of the triacrylic acid ester of the hydrogenated castor oil, which is easily soluble in most solvents. The chief constituent of the new ester corresponds to the formula



By heating it on the water-bath in the presence of a small quantity of benzoyl peroxide (for example, 0.1 per cent.) the new ester polymerises in a short time (3-10 minutes), yielding a horny friable mass. Instead of hardened castor oil octadecyl glycolate or the methyl ester of  $\alpha$ -hydroxy stearic acid or 11-hydroxy-stearic acid cetyl ester or the ricinoleic ester of stearic acid diglyceride may be used in a similar manner.

#### Example 2

A warm solution of 73 parts of castor oil in 230 parts of benzene is mixed with 18 parts of concentrated hydrochloric acid and 10 parts of nickel carbonyl, and the mixture is agitated with acetylene as described in Example 1. The whole is filtered to remove precipitated nickel chloride and heated for a further 2 hours at the boil while the water liberated during the reaction is separated with the aid of one of the known devices, and then the benzene is distilled off under reduced pressure.

78 parts of the triacrylic acid ester of castor oil remain behind in the form of an oil easily soluble in most solvents. The chief constituents of the new ester has the formula



By heating it on the water-bath in the presence of a small quantity of benzoyl peroxide (for example, 0.1 per cent.) a horny solid polymerisate is obtained in a short time.

#### Example 3

A solution of 164 parts of commercial stearic acid diglyceride in 260 parts of benzene having a temperature of 50-60° C. is agitated with acetylene with the addition of 18 parts of concentrated hydrochloric acid (density=1.199) and 10 parts of nickel carbonyl. When the gas is no longer absorbed, the mixture is worked up as described in Example 2.

## 5

There are obtained 159-160 parts of the acrylated diglyceride of the formula:



(wherein:



is the acyl radical of commercial stearic acid), which is a stiff mass after being cooled. It melts easily when heated on the water-bath, and dissolves well in the usual solvents. Upon the addition of a small quantity of benzoyl peroxide (for example, 0.1 per cent) a viscous oil is gradually formed, which upon further heating (1/2-1 hour) is converted into a slimy, slightly gelatinous product. At ordinary temperature the resulting polymerisate is solid and somewhat harder than the starting material, but rather sparingly soluble in organic solvents.

## Example 4

115.4 parts of a diglyceride (molecular weight about 493) obtained by the reaction of commercial linseed oil with glycerine are dissolved in 175 parts of benzene and, after the addition of 18 parts of concentrated hydrochloric acid (density=1.199) and 10 parts of nickel carbonyl, the solution having a temperature of 50-60° C. is agitated with acetylene until the gas is no longer absorbed.

After working up the product as described in Example 2 there are obtained 100 parts of an easily mobile oil, which after being heated on the water-bath for about 3/4-1 hour with the addition of a small quantity of benzoyl peroxide is converted into a soft, brittle, trituratable polymerisate. In a similar manner a diglyceride from benzoic acid may be used as starting material.

## Example 5

42 parts of commercial glycerine mono-stearate are dissolved in 135 parts of benzene having a temperature of 50-60° C., and then mixed with 18 parts of concentrated hydrochloric acid (density=1.199) and 10 parts of nickel carbonyl and agitated with acetylene. When the absorption of the gas has ceased, the whole is filtered, and the reaction solution is heated for 2 hours at the boil under reflux and while separating the water produced during the reaction. The solvent is then removed by distillation under reduced pressure leaving as a residue 42.5 parts of the acrylated product. After cooling, the resulting mono-stearic acid diacrylic acid glyceride of the formula



(wherein:



is the acyl radical of commercial stearic acid) is salve-like and easily soluble in most solvents. When heated for a short time on the water-bath after the addition of a small quantity of a polymerisation catalyst (for example, 0.1 per cent of benzoyl peroxide), the easily mobile oil changes into a stiff insoluble polymerisate. It can be used for rendering textiles water repellent.

## 6

## Example 6

87 parts of commercial ricinoleic acid and 100 parts of an ordinary commercial mixture consisting predominantly of octadecyl alcohol and a smaller quantity of cetyl alcohol are heated in the presence of 160 parts of benzene and 5.5 parts of concentrated sulfuric acid (density=1.84) for 6 hours at the boil in a reflux apparatus, while the condensate is allowed to return to the esterification vessel after passing through a water-removing device.

The reaction product is neutralised with calcium carbonate and a small quantity of sodium carbonate solution, filtered while warm, and used directly for acrylation.

One half of the solution of the ricinoleic acid ester prepared as described above, which contains about 100 parts of the ester, is heated to 50-60° C., then mixed with 18 parts of concentrated hydrochloric acid (density=1.199) and 10 parts of nickel carbonyl, and immediately agitated with acetylene. When the absorption of the gas has ceased, the filtered reaction product is heated under reflux for 2 hours, while the water split off during the esterification is removed from the condensate returning to the esterification vessel by means of a water-removing device. The solvent is then removed by distillation under reduced pressure. There remain as a residue 82.9 parts of the new ester in the form of a pale brown oil. It consists of a mixture of the ester of the formula



and of the ester of the formula:



45 By heating the easily mobile oil for about 2-3 hours on the water-bath in the presence of a small quantity of benzoyl peroxide (for example, 0.1 per cent) it is converted into a very viscous oil, which is resinous after being cooled. The 50 polymerisate dissolves fairly well in organic solvents such as benzene, etc.

## Example 7

A solution, heated to 40-50° C., of 80 parts of 55 ricinoleic acid isopropyl ester (boiling at 195-206° C. under 5 mm. pressure) in 135 parts of benzene is mixed with 18 parts of concentrated hydrochloric acid (density=1.199) and 10 parts of nickel carbonyl. The mixture is agitated with 60 acetylene until gas is no longer absorbed. After cooling the whole is filtered and further treated in the manner described in Example 6.

The resulting O-acrylic acid ricinoleic acid isopropyl ester may be purified by distillation under 65 a high vacuum. In addition to an undistillable residue of a polymeric product, it is obtained in a yield of 65 per cent., and boils at 179-187° C. under 0.1 mm. pressure.

The polymerisate is a viscous oil or a resin depending on the period of polymerisation.

## Example 8

100 parts of commercial sodium stearate are converted into the ethylene glycol monostearic acid ester by being heated with 100 parts of eth-

ylene chlorhydrin and 83 parts of decalin with the addition of 10 parts of sodium iodide.

When recrystallised from methanol and a small quantity of acetone, ethyl acetate or petroleum ether the ester melts at 63.5–64 °C.

A warm mixture of 77 parts of ethylene glycol monostearic acid ester in 175 parts of benzene is agitated with acetylene in the manner described in Example 1 with the addition of 18 parts of concentrated hydrochloric acid (density=1.199) and 10 parts of nickel carbonyl until the gas is no longer absorbed. After working up in the manner described in Example 6, there are obtained 83 parts of stearic acid acrylic acid ethylene glycol ester of the formula



wherein



is the acyl radical of commercial stearic acid.

The new ester is a salve-like mass and dissolves well in most solvents. By mixing the ester, liquefied by slightly heating it, with a small quantity of benzoyl peroxide (for example, 0.1 per cent.) it is converted after being heated for a short time (about 6-8 minutes) into a viscous oil, which after being further heated on the water bath ( $\frac{3}{4}$ -1½ hours) forms a jelly. When cold the polymerisate is wax-like. When highly polymerised it is practically no longer soluble in any organic solvents and merely swells therein. Instead of ethylene glycol monostearic acid ester another ester of ethylene glycol, for instance, the lauric acid ester or the capric acid ester may be used. Moreover, in the above reaction the hydrochloric acid may be replaced by anhydrous acetic acid.

### Example 9

92 parts of montanic acid (acid number=146.4, saponification number=175.2, and ester number=28.8), are dissolved with heat in 50 parts of alcohol and 175 parts of benzene, and a warm solution of 9.6 parts of sodium hydroxide in 20 parts of water and 50 parts of alcohol is then added to the hot solution while stirring strongly.

The mixture which immediately becomes stiff is evaporated to dryness, finally at 100° C. under reduced pressure.

100 parts of sodium montanate are heated gradually to 120° C., while stirring, with 80 parts of ethylene chlorhydrin in 130 parts of decalin with the addition of 10 parts of sodium iodide. The whole is stirred for 16 hours at 120-125° C. The mass which is at first pasty becomes thinly fluid as sodium chloride separates. The reaction mixture is filtered while hot, residual sodium chloride is removed by washing with hot decalin, and the united solutions are freed from excess of glycol chlorhydrin and solvent by distillation. The residual oil solidifies to a stiff mass after cooling. The yield amounts to 99-100 parts.

96 parts of the ethylene glycol monomontanic acid ester are dissolved in 265 parts of benzene with heat and, after the addition of 18 parts of concentrated hydrochloric acid (density=1.199) and 10 parts of nickel carbonyl, agitated with 70 acetylene in the manner described in Example 1 until gas is no longer absorbed. The whole is filtered hot to remove precipitated nickel chloride, and boiled for 2 hours under reflux as described in Example 6. The solvent is then removed by 75

distillation under reduced pressure. After cooling, there are obtained 94 parts of a wax-like substance. The montanic acid acrylic acid glycol ester melts when moderately heated on the water bath and is easily converted into an infusible polymeric mass by the addition of a small quantity of benzoyl peroxide (for example, 0.1 per cent.), which mass is no longer soluble in organic solvents.

*Example 10*

60.5 parts of an ordinary commercial mixture consisting predominantly of octadecyl alcohol and a small quantity of cetyl alcohol (hydroxyl number=217 and saponification number=0) are dissolved in 135 parts of benzene. 18 parts of concentrated hydrochloric acid (density=1.199) and 10 parts of nickel carbonyl are then added to the solution having a temperature of about 60° C.

The warm mixture is agitated with acetylene as described in Example 1 until gas is no longer absorbed. After cooling, the solid precipitated nickel chloride is removed by filtration and the solution is heated for 2 hours under reflux and with removal of the water liberated during the reaction, whereby the small quantity of free acrylic acid formed as a by-product is also esterified. The solvent is then removed by distillation under reduced pressure, and the residual oil may be distilled under a high vacuum. After separating a small amount of material which distils initially, the new acrylic acid ester, a mixture of



and



distills under 0.1 mm. pressure at 145-169° C. and is a colorless mass after being cooled. The yield amounts to 51 parts.

*Example 11*

70 parts of commercial ricinoleic acid are dissolved in 135 parts of benzene heated at 50-60° C., then mixed with 18 parts of concentrated hydrochloric acid (density=1.199) and 10 parts of nickel carbonyl, and at the same time agitated with acetylene until gas is no longer absorbed. The cooled reaction liquid is filtered and then the acrylic acid formed as a by-product is esterified by boiling the reaction liquid for 2 hours under reflux while removing water.

After removing the benzene by distillation under reduced pressure there are obtained 77 parts of a pale brown oil which is gradually converted into a viscous oil by heating it on the water bath in the presence of a polymerisation catalyst. The polymerisate still dissolves quite well in organic solvents, for example benzene. The chief constituent of the monomer corresponds to the formula



*Example 12*

A mixture, heated at about 40° C., of 90 parts of dodecylalcohol (boiling at 142–147° C. under 13 mm. pressure), 36 parts of concentrated hydrochloric acid (density=1.199) and 20 parts of nickel carbonyl is agitated with acetylene under

an absolute pressure of 1½ atmospheres of acetylene until gas is no longer absorbed. When 1½-2 hours have elapsed and 10-11 parts by volume of acetylene have been absorbed the reaction ceases.

The reaction product is extracted with water, the aqueous solution containing the nickel salt is separated and the crude ester is repeatedly washed water and a normal solution of sodium bicarbonate. In order to obtain a better separation it is recommended after the treatment with the alkaline washing liquid, to add petroleum ether, a small quantity of concentrated sodium chloride solution and a very small quantity of phosphoric acid.

The crude ester is obtained, after drying with sodium sulfate and distilling off any added solvent under reduced pressure, in a yield of 106.5 parts.

For further purification the product may be fractionally distilled under a high vacuum. The pure ester of the formula



boils at 121-138° C. under 0.07-0.15 mm. pressure. Instead of hydrochloric acid anhydrous acetic acid may be used.

#### Example 13

(a) 2 parts of the acrylic acid montanic acid ethylene glycol ester described in Example 9 are mixed with 2 parts of the acrylic acid distearic acid glycerine ester described in Example 3 with heat and occasional stirring and heated, after the addition of 0.04 part of benzoyl peroxide, at 95-100° C. until the oil begins to become thickly liquid (about 3-9 minutes).

The resulting polymerisate is immediately dissolved in 40 parts of benzene, and a fibrous material, for example, a cotton fabric is impregnated with the solution. The product remaining on the fiber after evaporation of the solvent is after-polymerised by heating the treated material for 1 hour, whereby a water-repellent dressing is produced which is substantially unaffected by washing with aqueous baths and by treatment with organic solvents. Furthermore, the fabric finished in this manner has a soft full feel.

(b) A mixture of 5 parts of acrylic acid stearic acid ethylene glycol ester described in Example 8 and 5 parts of the triacrylic acid ester of hardened castor oil described in Example 1 is mixed while stirring and heating on the water bath with 0.1 part of benzoyl peroxide, which is advantageously added in solution in a small quantity of benzene. The resulting oil is then dissolved in 100 parts of benzene and a fibrous material, for example, cotton gaberdine or poplin, is then impregnated with the solution. After squeezing the material and evaporating the solvent, the material is heated for one hour at 120° C., whereby the substance is polymerised on the fiber and rendered insoluble.

The fabric so treated has a water-repellent finish similar to that of the material treated as described under (a) above.

Having thus described the invention, what is claimed is:

1. A process for the manufacture of an acrylic acid ester which comprises treating acetylene with nickel carbonyl with the addition of an acid and of a hydroxy compound which contains at least one alcoholic hydroxy group and at least

one carbon chain with at least 12 carbon atoms, in the presence of water and of a water-insoluble organic solvent selected from the group consisting of hydrocarbons of the benzene series, hydrocarbons of the benzene series and mixtures thereof.

2. A process for the manufacture of an acrylic acid ester which comprises treating acetylene with nickel carbonyl with the addition of an acid

10 and of dodecyl alcohol, in the presence of water and of a water-insoluble organic solvent selected from the group consisting of hydrocarbons of the benzene series, hydrocarbons of the benzene series and mixtures thereof.

15 3. A process for the manufacture of an acrylic acid ester which comprises treating acetylene with nickel carbonyl with the addition of aqueous hydrochloric acid, of a water-insoluble organic solvent selected from the group consisting of hydrocarbons of the benzene series, hydrocarbons of the benzene series and mixtures thereof and of dodecyl alcohol under an acetylene pressure which exceeds one atmosphere.

20 4. A process for the manufacture of an acrylic acid ester which comprises treating acetylene with nickel carbonyl with the addition of an acid and of a partial ester of a polyhydric alcohol with an aliphatic carboxylic acid containing at least 12 carbon atoms, in the presence of water and of a water-insoluble organic solvent selected from the group consisting of hydrocarbons of the benzene series, hydrocarbons of the benzene series and mixtures thereof.

25 5. A process for the manufacture of an acrylic acid ester which comprises treating acetylene with nickel carbonyl with the addition of an acid and of glycerine-monostearate, in the presence of water and of a water-insoluble organic solvent selected from the group consisting of hydrocarbons of the benzene series, hydrocarbons of the benzene series and mixtures thereof.

30 6. A process for the manufacture of an acrylic acid ester which comprises treating acetylene with nickel carbonyl with the addition of an acid and of stearic acid-β-hydroxyethyl ester, in the presence of water and of a water-insoluble organic solvent selected from the group consisting of hydrocarbons of the benzene series, hydrocarbons of the benzene series and mixtures thereof.

35 7. A process for the manufacture of an acrylic acid ester which comprises treating acetylene with nickel carbonyl with the addition of an acid and of an ester of an aliphatic hydroxycarboxylic acid containing 18 carbon atoms, in the presence of water and of a water-insoluble organic solvent selected from the group consisting of hydrocarbons of the benzene series, hydrocarbons of the benzene series and mixtures thereof.

40 8. A process for the manufacture of an acrylic acid ester which comprises treating acetylene with nickel carbonyl with the addition of an acid and of castor oil, in the presence of water and of a water-insoluble organic solvent selected from the group consisting of hydrocarbons of the benzene series, hydrocarbons of the benzene series and mixtures thereof.

45 9. A process for the manufacture of an acrylic acid ester which comprises treating acetylene with nickel carbonyl with the addition of an acid and of an ester of hardened ricinoleic acid, in the presence of water and of a water-insoluble organic solvent selected from the group consisting of hydrocarbons of the benzene series, hydrocarbons of the benzene series and mixtures thereof.

11

10. A process for the manufacture of an acrylic acid ester which comprises treating acetylene with nickel carbonyl with the addition of an acid and of hardened castor oil in the presence of water and of a water-insoluble organic solvent selected from the group consisting of hydrocarbons of the benzene series, hydrocarbons of the benzine series and mixtures thereof.

OTTO ALBRECHT.  
ARTHUR MAEDER.

12

## UNITED STATES PATENTS

| Number    | Name   | Date          |
|-----------|--------|---------------|
| 2,141,546 | Strain | Dec. 27, 1938 |

## 5 OTHER REFERENCES

5 Modern Plastics, November 1945, pages 162, 163 and 210.

10 Reppe: Advances in Acetylene Chemistry, Enemy Technical Information, Intelligence Div.

10 Report No. 4149, February 12, 1946, pages 21-23.

## REFERENCES CITED

The following references are of record in the file of this patent: